



US011008263B2

(12) **United States Patent**  
**Isert et al.**

(10) **Patent No.:** **US 11,008,263 B2**  
(45) **Date of Patent:** **May 18, 2021**

(54) **REACTIVE BURNING RATE ACCELERATORS, SOLID ENERGETIC MATERIALS COMPRISING THE SAME, AND METHODS OF USING THE SAME**

(71) Applicant: **PURDUE RESEARCH FOUNDATION**, West Lafayette, IN (US)

(72) Inventors: **Sarah Isert**, Abingdon, MD (US); **Steven Forrest Son**, West Lafayette, IN (US); **Colin D. Lane**, Odessa, FL (US); **Ibrahim Emre Gunduz**, Lincoln, NE (US)

(73) Assignee: **Purdue Research Foundation**, West Lafayette, IN (US)

(\*) Notice: Subject to any disclaimer, the term of this patent is extended or adjusted under 35 U.S.C. 154(b) by 517 days.

(21) Appl. No.: **15/423,877**

(22) Filed: **Feb. 3, 2017**

(65) **Prior Publication Data**

US 2018/0022663 A1 Jan. 25, 2018

**Related U.S. Application Data**

(60) Provisional application No. 62/291,865, filed on Feb. 5, 2016.

(51) **Int. Cl.**

**C06B 45/14** (2006.01)  
**C06B 43/00** (2006.01)

(52) **U.S. Cl.**  
CPC ..... **C06B 45/14** (2013.01); **C06B 43/00** (2013.01)

(58) **Field of Classification Search**

None  
See application file for complete search history.

(56) **References Cited**

**U.S. PATENT DOCUMENTS**

|                   |        |                 |              |
|-------------------|--------|-----------------|--------------|
| 6,342,272 B1 *    | 1/2002 | Halliwell ..... | B05D 1/10    |
|                   |        |                 | 427/447      |
| 7,524,355 B2 *    | 4/2009 | Dreizin .....   | C06B 21/0066 |
|                   |        |                 | 148/513      |
| 9,227,883 B2 *    | 1/2016 | Sippel .....    | C06B 45/18   |
| 2010/0032064 A1 * | 2/2010 | Dreizin .....   | C06B 21/0066 |
|                   |        |                 | 149/37       |
| 2014/0034197 A1 * | 2/2014 | Sippel .....    | C06B 45/18   |
|                   |        |                 | 149/3        |

\* cited by examiner

*Primary Examiner* — Aileen B Felton

(74) *Attorney, Agent, or Firm* — Hartman Global IP Law; Gary M. Hartman; Domenica N. S. Hartman

(57) **ABSTRACT**

A reactive burning rate accelerator is provided that is configured to be at least partially embedded in a solid energetic material and comprises at least one metallic component and at least one non-metallic component. The reactive burning rate accelerator is configured to ignite and combust to increase the mass burning rate of the solid energetic material. Also provided are solid energetic materials comprising the reactive burning accelerator and methods of manufacturing and using the same.

**17 Claims, 12 Drawing Sheets**





FIG. 1



FIG. 2





FIG. 3



FIG. 4





FIG. 5



FIG. 6



FIG. 7



FIG. 8



FIG. 9



FIG. 10



FIG. 11



FIG. 12



FIG. 13

**REACTIVE BURNING RATE  
ACCELERATORS, SOLID ENERGETIC  
MATERIALS COMPRISING THE SAME, AND  
METHODS OF USING THE SAME**

**CROSS REFERENCE TO RELATED  
APPLICATIONS**

This application claims the benefit of U.S. Provisional Application No. 62/291,865, filed Feb. 5, 2016, the contents of which are incorporated herein by reference.

**STATEMENT REGARDING FEDERALLY  
SPONSORED RESEARCH**

This invention was made with government support under Contract No. FA9550-13-1-0004 awarded by the Air Force Office of Scientific Research, and under Contract No. 1147384 awarded by the National Science Foundation Graduate Fellowship Program. The government has certain rights in the invention.

**BACKGROUND OF THE INVENTION**

The present invention generally relates to solid propellants energetic materials and reactive burning rate accelerators for use therewith. The invention particularly relates to solid energetic materials comprising reactive burning rate accelerators, methods for their manufacture, and methods for their use.

Solid propellants commonly used in rockets and aircraft are used in forms referred to as propellant charge (grains) made up of a fuel and an oxidizer that causes the fuel to burn or otherwise decompose to produce a propellant gas. There are numerous factors which affect propellant performance, such as the propellant composition, its linear burning rate, its ambient temperature, combustion chamber pressure, and the like. A particularly important parameter that affects thrust of propellant grains, which are loaded into and burned directly in the combustion chamber of a rocket motor or engine, is the burning surface area, which greatly affects the mass rate of gas generation. The rate of generation of propulsive gases, other factors being equal, is proportional to the product of the propellant burning rate and the burning surface area. Tailoring solid propellant burning rates is a perpetual goal of solid propellant designers. Traditional approaches to tailoring propellant burning rates include modifying the particle size of the oxidizer and adding catalysts to the propellant. However, these methods only increase the propellant burning rate up to a certain point and can diminish propellant performance.

The addition of burning rate accelerators (or simply accelerators) to propellants has been used to improve and tailor burning rates. For example, inert metallic staples, whiskers, foils, and wires have been cast into the grain of propellants in order to increase propellant thermal conductivity and provide a low-resistance thermal path for heat flow from the flame into the propellant. Metallic accelerators have been used in various thicknesses, lengths, and shapes. Relatively short staples, whiskers, fibers, and the like are commonly randomly distributed throughout solid propellant grains. Wires are typically distributed as long strands embedded axially in solid propellant grains. Wired propellants in particular have been used in thousands of fielded sounding rockets and tactical missiles.

Inert metallic accelerators cause local preheating that results in locally increased burning rates and changes the

burning surface profile to cause increased overall mass burning rate. However, inert metallic accelerators, and wires in particular, can sometimes act as heat sinks and decrease propellant burning rate and performance. As such, inert metallic accelerators generally increase burning rate only if the volume and weight fractions are adequately low. Consequently, such accelerators provide only a limited range of burning rate augmentation.

When a propellant grain includes inert metallic wires as an accelerator, the embedded wires cause an increase in surface area as the burning surface transforms from a nominally flat surface to a cone-like surface. Generally, the cone-like burning surface forms when multiple burning rates are present, and the fastest burning rate dominates the process. At steady-state, the constant thrust profile of an end-burner motor may be retained but the mass burning rate of the propellant will likely be higher. Commonly used inert wires include copper, silver, silver alloys, steel, tungsten, aluminum, magnesium, nickel, molybdenum, brass, platinum, and relatively low melting point metals plated with higher melting point metals.

The degree of burning rate enhancement from embedded wire accelerators depends on wire thermal diffusivity and melting temperature. For long wires, burning rate generally increases with increasing wire diameter up to a certain point, after which it decreases as thermal sink losses become more significant. Cross-sectional shape of wire accelerators has been reported to weakly affect burning rate as long as the length-to-diameter ratio is relatively high.

Despite the advantages of inert metallic burning rate accelerators, several factors limit their performance. For example, embedded wires may cause an overall performance decrease if the wire acts as a heat sink to the propellant. In addition, casting long, straight axial wires can be difficult, and non-uniform wire spacing may cause unintended thrust profiles as the propellants regress. In regards to fibers, whiskers, staples, etc., poor bonding between the accelerators and the propellant may cause grain cracking, and thermal cycling may cause de-bonding between the grain and fibers.

Non-metallic burning rate accelerators have also been attempted. For example, propellant grains comprising embedded optical fibers have been used in laser-assisted combustion, and Kevlar® fibers have been observed to act as flame holders and can affect the burning rate.

Self-alloying systems such as nickel/aluminum foils or aluminum-palladium core-shell wires (commercially available under the trademark Pyrofuz® from Pyrofuz Corp.) have been proposed for use in propellant grains. Self-alloying wires may increase a propellant's burning rate; however, self-alloying wires may decrease the specific impulse of the propellant considerably compared to propellant grains with aluminum as an accelerator, and even slightly compared to propellants without an accelerator. Specific impulse is the total impulse (or change in momentum) delivered per unit of propellant consumed and is dimensionally equivalent to the generated thrust divided by the propellant flow rate.

Therefore, other approaches are needed to tailor burning rates of propellants over a wider range than conventionally possible in order to enable the design of currently unattainable rocket solid propellant grain configurations.

**BRIEF DESCRIPTION OF THE INVENTION**

The present invention provides reactive burning rate accelerators suitable for improving mass burning rates of

solid energetic materials, solid energetic materials comprising the same, and methods of using the same.

According to another aspect of the invention, a reactive burning rate accelerator is provided that is configured to be at least partially embedded in a body comprising a solid energetic material and comprises at least one metallic component and at least one non-metallic component. The reactive burning rate accelerator is configured to ignite and combust to increase the mass burning rate of the solid energetic material.

According to one aspect of the invention, a body formed of a solid energetic material is provided that includes a reactive burning rate accelerator at least partially embedded in the body. The reactive burning rate accelerator comprises a mechanically-activated material that is at least partially formed of micron-sized particles comprising nano-thickness layers of at least one metallic component and at least one non-metallic component. The reactive burning rate accelerator is configured to ignite and combust to increase the mass burning rate of the solid energetic material.

According to another aspect of the invention, a method of combusting a solid energetic material is provided that includes igniting a reactive burning rate accelerator embedded in a body formed of the energetic material. The reactive burning rate accelerator comprises a material that is at least partially formed of micron-sized particles comprising nano-thickness layers of at least one metallic component and at least one non-metallic component. The reactive burning rate accelerator is configured to ignite and combust to increase the mass burning rate of the solid energetic material.

Technical effects of reactive burning rate accelerators of types described above preferably include the ability to improve the mass burning rate and specific impulse of solid energetic materials, such as solid propellants, relative to conventional burning rate accelerators.

Other aspects and advantages of this invention will be further appreciated from the following detailed description.

#### BRIEF DESCRIPTION OF THE DRAWINGS

FIGS. 1 and 2 each include cross-sectional and perspective views that schematically represent reactive burning rate accelerators embedded in solid energetic material bodies in accordance with certain nonlimiting aspects of the invention.

FIG. 1 includes a single reactive burning rate accelerator in the energetic material and

FIG. 2 includes multiple reactive burning rate accelerators in the energetic material.

FIG. 3 schematically represents a cross-sectional view of a nonlimiting embodiment of a rocket comprising a solid propellant grain having a reactive burning rate accelerator embedded in the propellant.

FIG. 4 includes two images representing a propellant grain with an embedded wire, including a schematic representation of a top view of the propellant (left), and an image showing an actual cast propellant with a Pyrofuz® wire visible through a polycarbonate window.

FIG. 5 includes a series of time lapsed images representing the combustion of a propellant grain having a copper wire therein at 13.8 MPa with 80 ms between frames (progressing left to right).

FIG. 6 includes two images representing a propellant grain having a copper wire therein and exhibiting a burning surface cone angle of about 4.8 MPa (image a, left) and 19.3 MPa (image b, right).

FIG. 7 is a graph representing changes in burning surface cone angle as a function of pressure for embedded copper wire propellant grains.

FIG. 8 includes a series of time lapsed images representing the combustion of a nickel/aluminum foil propellant grain at 13.8 MPa with 20 ms between frames (progressing left to right). The propellant ignited within 20 ms of first contact with the hot wire.

FIG. 9 includes a series of time lapsed images representing the combustion of a Pyrofuz® wire propellant grain at 13.8 MPa with 40 ms between frames (progressing left to right).

FIG. 10 includes a series of time lapsed images representing combustion of a freestanding aluminum/polytetrafluoroethylene (Al/PTFE) strand burning at 1 atm with 76 ms between frames (progressing left to right).

FIG. 11 includes a series of time lapsed images representing combustion of a Al/PTFE foil propellant grain at 13.8 MPa with 80 ms between frames (progressing left to right). A flame appears above the reacting foil.

FIG. 12 is a graph representing changes in the burning rate of propellants near Al/PTFE foils as a function of pressure. Baseline propellant burning rate with 95% confidence bands is also shown.

FIG. 13 is an image showing slag from a copper wire propellant grain (top) and Ni/Al foil propellant grain (bottom) collected post-burn.

#### DETAILED DESCRIPTION OF THE INVENTION

The present invention generally provides reactive burning rate accelerators (reactive accelerators), for example, foils, wires, etc., in contact with and/or embedded into a solid energetic material, such as but not limited to explosives, propellants, pyrotechnics, and fuels, in order to increase the propellant mass burning rate. Reactive accelerators are defined herein as accelerators that exothermically react, combust, and burn by themselves when ignited and produce a source of heat, that is, once ignited at an ignition temperature, the temperature of the reactive accelerator increases to a combustion temperature at which it combusts and provides heat to the propellant to ignite it. In contrast, other accelerators discussed herein are inert, and while they may exothermically self-alloy, they do not exothermically react, combust, and burn by themselves when ignited. Once activated, the combustion of the reactive accelerators ignites the energetic material with which it is in contact, increasing the mass burning rate of the energetic material by exposing more burning surface area.

Preferably, the reactive accelerators not only increase the energetic material's burning rate, but are also an active participant in the material's combustion, adding gas pressure to the system and preferably leaving little or no condensed phase materials (referred to herein as slag), as would commonly result from inert and self-alloying wires/foil accelerators. Preferably, any reaction products, combustion products, or other condensed phase materials remaining after the combustion of the reactive accelerators have diameters (or maximum lengths, widths, and depths) of less than one millimeter, preferably up to 200 micrometers, and more preferably up to 10 micrometers (e.g., 0.1 nm-10  $\mu$ m). For convenience, the reactive accelerators will be primarily discussed herein in reference to solid propellants. However, the reactive accelerators may be used for various applications, including increasing the burning rate of a wide variety of explosives, propellants, pyrotechnics, and fuels. As a

nonlimiting example, the reactive accelerators may be used as a low temperature gas generator of the types commonly used in, for example, automotive safety devices, such as but not limited to airbags.

The reactive accelerators may be added to a propellant grain in various configurations or patterns and may have various cross-sectional shapes and lengths. For example, foil- or wire-shaped accelerators may be oriented axially through the center of a propellant grain, randomly mixed into a propellant grain, or embedded in a propellant grain according to a desired pattern. FIGS. 1 and 2 schematically represent reactive accelerators 12 embedded in solid energetic material bodies 10. FIG. 1 includes a single reactive accelerator 12 and FIG. 2 includes multiple reactive accelerators 12. FIG. 3 schematically represents a nonlimiting rocket 14 comprising solid propellant grain 16 having a single reactive accelerator 12 oriented axially through the center of the grain 16.

Propellants comprising the reactive accelerators may be formed by various means, including but not limited to those conventionally used for inert and self-alloying accelerators. For example, one or more reactive accelerators may be cast in a propellant grain, or may be formed/inserted into a propellant grain with a three-dimensional (3-D) printing process. The 3-D printing process can either be accomplished by sequential printing of the propellant and the reactive accelerator, or by printing of the propellant to encapsulate an already fabricated reactive accelerator, into the final desired geometry. The reactive accelerators described herein may be used with any suitable propellant, such as but not limited to non-aluminized ammonium perchlorate/hydroxyl-terminated polybutadiene (AP/HTPB) composite propellants as discussed in the investigations below, as well as other solid propellants, including but not limited to composite solid propellants, double-base solid propellants, and composite double-base solid propellants.

The reactive accelerator may have various compositions. According to one nonlimiting embodiment of the invention, a reactive accelerator comprises at least one metallic component and at least one non-metallic component. Preferably, the reactive accelerator is mechanically-activated, that is, the components of the accelerator are combined mechanically using a technique such as, but not limited to, arrested reactive milling, to preferably result in micron-sized particles formed of nano-thickness layers of the components. As used herein, the term micro-sized particles denote particles having a diameter (or maximum length, height, and width) of about 1 to 999 micrometers, and more preferably about 10 to 50 micrometers, and the term nano-thickness layers denote layers of a layer having at least one dimension of less than one micrometer, and preferably up to 200 nanometers, and more preferably up to 100 nanometers, e.g., 0.1-100 nm.

Nonlimiting examples of mechanical-activation processes are disclosed in U.S. Patent Application Serial No. 2010/0032064 to Dreizin et al. and U.S. Pat. No. 9,227,883 to Sippel et al. In such processes, the fineness (thickness) of the layers generally provides the mechanically-activated material with a high reactivity. In contrast, conventional milling of the components to micron-sized particles generally would not produce particles formed of multiple components. Therefore, the components may have relatively long diffusion distances (on the order of microns rather than nanometers), yielding slower reaction times and less vigorous reactions. Conventionally produced nano-sized particles (that is, particles having a diameter (or maximum length, height, and width) of about 10 to 200 nanometers) may have diffusion

distances similar to micron-sized mechanically-activated particles, but such nano-sized particles can be difficult to handle as they are very reactive. With the mechanically-activated materials, the particles have nano-thickness layers (features) that have short diffusion distances, but the particles themselves are micron-sized and therefore are likely to be more stable and safer to handle than nano-sized particles.

The reactive accelerator may include the at least one metallic component and at least one non-metallic component 10 in various amounts, and may consist essentially of the metallic and non-metallic components (perhaps with incidental impurities) or may comprise additional components. Suitable materials may comprise a metallic component and a non-metallic component that in combination can self-react 15 exothermically, that is, doesn't require an external oxidizer, and that once ignited locally, can continue to react until substantially all of the material combusts and is consumed and preferably produces a gas. Suitable non-metallic components may include, but are not limited to, materials 20 comprising various oxides, nitrides, chlorides, carbides, and fluorides that are capable of being exothermically reduced with a corresponding metallic component. Such materials may be contained in polymeric materials. It is foreseeable that the MA reactive accelerators may comprise particles 25 that consist of only one metallic component and one non-metallic component (perhaps with incidental impurities).

For example, one nonlimiting reactive accelerator suitable 30 for use in solid propellants is a mechanically-activated (MA) aluminum-rich aluminum/polytetrafluoroethylene (Al/PTFE) accelerator, wherein the manufacturing process results in the accelerator comprising nanoscale features 35 (e.g., nano-thickness layers within individual micron-sized particles). Suitable compositions of the Al/PTFE accelerator may include between 50 to 90 wt. % Al with the remainder being PTFE. Combustion products of the accelerator include relatively small (for example, less than about 10 micrometers in diameter) aluminum droplets and carbon, which can burn to increase the gas temperature and gas volume of the system. It is believed that the closer the percentages are to 40 stoichiometric combustion, the more reactive the particles will be. Additionally, the burning rate of the accelerators may change as the composition changes, leading to an ability to tailor the burning rate of the propellant. Another exemplary composition for the reactive accelerator includes 45 an aluminum/poly(carbon monofluoride) (Al/PMF) accelerator comprising between 70 to 90 wt. % Al, the remainder being poly(carbon monofluoride) (PMF). Similar to PTFE, PMF contains fluorine which is a powerful oxidizer, and provides exothermic heat generation when reacted with a 50 metal, in this instance, aluminum.

The reactive accelerators described herein are believed to 55 increase the efficiency of propellants as compared to inert and self-alloying accelerators. By using reactive accelerators in a propellant grain, the propellant ignition rate may be significantly increased as the flame front along the reactive accelerator propagates at an increased rate compared to the flame front of a propellant that does not include an accelerator, or even a propellant grain having an inert or self-alloying accelerator. Igniting the propellant at the flame 60 front along the reactive accelerator causes the propellant to regress away from the accelerator as well as in the bulk axial direction of the overall propellant combustion. This causes an increase in surface area of the propellant that is exposed near the flame front which results in an overall increase in the mass burning rate. Furthermore, reaction products (for example, aluminum and carbon) are formed from the combustion of the reactive accelerators. These products may 65

oxidize with propellant combustion products and increase the temperature of the combustion gases. In addition, the products may include significant amounts of gas that is released into the system. Because the reactive accelerators contribute to the energy and gas production of the propellant, the specific impulse of the propellant may be improved compared to propellants that do not comprise burning rate accelerators, or even compared to propellant grains having an inert or self-alloying accelerator.

In addition, inert and self-alloying wire/foil accelerators often deposit slag post-combustion that may increase two-phase flow losses of propellants. In contrast, preferred reactive accelerators of the present invention preferably burn completely and leave little or no slag or other left over materials. As such, the reactive accelerators may result in a decrease in slag production compared to inert and self-alloying wires/foil accelerators.

Reactive accelerators as described herein are believed to be well suited for use in solid propellants due to the high burning rate tailorability and their participation in propellant combustion. It is foreseeable that the overall mass burning rate of a propellant may be prescribed by the type of reactive accelerator used and the number and location of the accelerators. It is believed that adding reactive accelerators to propellant grains has the potential to create more efficient rockets as center perforations (that is, cavities provided within the grain to increase surface area) could be created in situ rather than cast into the propellant as is customary. This would result in dramatically increased propellant loading for the same overall rocket volume. Additionally, the addition of reactive accelerators into rocket solid propellant grains may allow for increased tailorability of solid rocket ballistics. Tailoring of the mass burning rate may be accomplished over a wide range by, for example, adjusting the ratio of the metallic and non-metallic components in the reactive accelerator, modifying the mechanical activation conditions, considering other inclusion materials or metals, etc.

Nonlimiting embodiments of the invention will now be described in reference to experimental investigations leading up to the invention. The following investigations examined the burning rates of exothermically alloying nickel/aluminum foils, Pyrofuz® wires, and pressed foils made from mechanically-activated aluminum/polytetrafluoroethylene (Al/PTFE). The observed burning rates were compared to propellant grains comprising embedded inert copper wires.

For the investigations described herein, non-aluminized ammonium perchlorate/hydroxyl-terminated polybutadiene (AP/HTPB) composite propellants with 80 wt. % solids loading and a 1:1 bimodal oxidizer size distribution with 400 micrometer coarse AP (Firefox Enterprises) and 20 micrometer fine AP (ATK) were used as solid propellants. The propellants included R45-M prepolymer (Firefox Enterprises) with Tepanol HX-878 bonding agent (3M Corporation) as a binder, icodecyl pelargonate plasticizer (RCS RMC), and Desmodur E744 curative (Bayer Corporation). The propellants were hand-mixed, degassed for ten minutes under vacuum, and cast into molds.

Four metallic fibers were investigated including copper wire, nickel/aluminum foils, Pyrofuz® wire, and Al/PTFE foils. The 20 gage copper wires (0.81 mm diameter) had a round cross-section. The nickel/aluminum nanofoil (NF80, Indium Corporation) were 80 micrometers thick and consisted of nanoscale alternating layers of nickel and aluminum. When this type of foil is ignited, it exothermically self-alloys. The cut foils were approximately 1 mm×80 µm×25.4 mm in size. The Pyrofuz® wire (0.007 inch

diameter, Sigmund-Cohn Corporation) consisted of an inner aluminum core and an outer shell of 95 wt. % palladium/5 wt. % ruthenium. Once ignited, Pyrofuz® wire alloys exothermically. The approximate minimum ignition temperature is 650° C. and the alloying reaction temperature is about 2800° C.

Mechanically-activated Al/PTFE (70/30 wt. %) foil was prepared to have sieved particle diameters of between 25 and 75 micrometers. To create the foils, 0.82 g of material 10 was remotely pressed on a Carver press (model NBS-400) at 34.5 MPa for 5 minutes in a square custom-built 25×25 mm die. The pressed foils were cut using a razor blade into 1 mm strands, resulting in 1 mm×1 mm×25.4 mm pressed Al/PTFE strands.

As it was desired to see how embedded wires affect the propellant surface, and as the AP/HTPB propellant was opaque, a windowed design was used. Although a window 15 may slightly affect propellant burning rate, it beneficially allowed direct visualization of the burning surface. The 20 propellants were cast in two-part molds. Polycarbonate windows were placed upright in the molds that were then filled half-way with propellant. The wire or foil was placed directly against the window. The mold was then filled completely with propellant, covering the wire. A diagram of 25 a representative sample can be seen in FIG. 4 (left) comprising the solid propellant grain 10, reactive accelerator 12, and window 18, and an actual sample containing a Pyrofuz® wire can be seen in FIG. 4 (right).

Propellants were ignited with Nichrome wire and burned 30 in a nitrogen-pressurized strand burner at pressures between 4.8 and 19.3 MPa. Multiple samples were burned at each pressure level and image data were collected using a high-speed camera operating at 2000-2500 fps. Propellant burning rates were determined from the videos. As the propellant 35 burned, the polycarbonate window accumulated char. However, the window in front of the unburned propellant remained clear such that the regression of the propellant surface was readily visible and the propagation of the flame front could be tracked. For some tests, slag from the copper 40 and Ni/Al wires was collected. Pressed Al/PTFE foils were also epoxide to a stand and ignited in air using a CO<sub>2</sub> laser.

FIG. 5 is a series of time lapsed images representing an 45 embedded copper wire propellant grain burning at 13.8 MPa. The wire is visible as a dark colored region through a center portion of the light colored propellant. A cone-shape cavity can be seen developing as the propellant burns. Though not visible in these images, there was a slight delay between the glowing wire being heated and the propellant igniting. The propellant burned axially as well as laterally from the wire surface. Remaining copper wires were often recovered post-test after the propellant had burned completely.

The ignition front of the burning copper wire propellant 50 grain was observed to move at an average speed of 28.6±4.51 mm/s over all pressures investigated. The cone half-angle formed was believed to be

$$\theta = \alpha \sin(r_{bo}/r_{be})$$

where  $r_{bo}$  is the bulk propellant burning rate and  $r_{be}$  is the 55 enhanced burning rate at the tip of the cone. The half-angle at which the propellant burned away from the wire changed from about 10° at 4.8 MPa to about 21° at 19.3 MPa, very similar to the half-angles calculated from prediction models. The change in cone angle was believed to be a result of the 60 flame front of the propellant near the wire traveling at a constant velocity regardless of pressure while the bulk propellant burning rate increased with pressure. Conse-

quently, at higher pressures the cone angle was larger because the propellant was regressing faster away from its ignition point. The change in cone angle can be seen visually for propellants at 4.8 and 19.3 MPa in FIG. 6 (image a and b, respectively) and graphically in FIG. 7.

Nickel/aluminum (Ni/Al) nanoscale foil is an exothermically self-alloying material that was chosen as a good contrast to inert and gas-producing reactive wires. FIG. 8 is a series of time lapsed images representing a typical burn progression of a Ni/Al foil propellant grain observed during the investigations. The foil is visible as a dark colored region through a center portion of the light colored propellant. The self-alloying reaction proceeded quickly and ignited the propellant as the alloying reaction passed by. After ignition, the propellant burned at the pressure-dependent bulk propellant rate (FIG. 12). Large pieces of remaining alloyed product from the Ni/Al foils were frequently found post-burn.

The Ni/Al foils reacted at  $5900 \pm 700$  mm/s over all pressures investigated. The burning rate is stated by the product literature as 6500-8000 mm/s. The decrease in the burning rate observed was believed to be due to heat loss into the window and the surrounding propellant. The reaction velocity of such foils can be tailored and is expected to change with foil bilayer thickness. Unlike the copper-wired propellant grains, the burning surface angles (cone half-angles) of the Ni/Al propellant grains were constant and relatively small ( $2.91 \pm 0.64^\circ$ ) though slightly larger than predicted. The difference between the observed and theoretical angles was believed to be due to factors such as augmented heating and the foils not being perfectly perpendicular.

NASA CEA calculations were performed for a rocket with a propellant grain comprising about 70 wt. % AP, 14 wt. % HTPB, 8 wt. % Al, and 8 wt. % Ni (i.e., Ni/Al foil accelerator). The vacuum specific impulse was decreased by about 8% compared to an equivalent propellant grain with 16 wt. % Al (i.e., Al foil accelerator). The nickel and aluminum alloying temperature was predicted to be about 1800 K, which is lower than aluminum combustion temperatures, and the products were higher in molecular weight, decreasing the specific impulse. The Ni/Al propellant grain was calculated to have a specific impulse that was 1.6% lower than a non-aluminized propellant grain containing about 86 wt. % AP and 14 wt. % HTPB (i.e., no accelerator).

Pyrofuzer® wire is widely used in industry to ignite energetic materials, including explosives, propellants, and pyrotechnics. During the investigations, the self-alloying propagation speed was measured to be  $85.3 \pm 13.2$  mm/s inside the propellant at the tested pressures compared to a reported value of 200 mm/s at 1 atm and a measured value of  $330 \pm 25$  mm/s at 1 atm. Again, it is believed that these differences were due to heat loss to the surrounding propellant and window. FIG. 9 is a series of time lapsed images representing a typical burn progression of a Pyrofuzer® wire propellant grain observed during the investigations. The wire is visible as a relatively thin, dark-colored region through a center portion of the light-colored propellant. The propellant burning surface angle was constant at  $3.98 \pm 0.64^\circ$ , which was larger than the theoretical value. The increased heat transfer from the hot wire may explain why the cone angles were similar between the Pyrofuzer® wire and Ni/Al foil propellant grains even though the enhanced burning rates were an order of magnitude different.

At 1 atm, Al/PTFE foils readily burn independently and produce small particles. FIG. 10 is a series of time lapsed images representing a burn progression of a free-standing

Al/PTFE foil observed during the investigations. The foil is visible as a dark-colored region in the images and smaller particles can be seen near the flame at an uppermost portion of the foil. The burning rate was measured to be approximately 20 mm/s. These foils were also placed in propellant grains and studied. FIG. 11 is a series of time lapsed images representing a burn progression of a Al/PTFE foil propellant observed during the investigations. The foil is visible as a dark-colored region through a center portion of the light-colored propellant. The foil was observed as burning independently as well as igniting the propellant. As pressure increased, no substantial change in the cone angle was observed. It is believed that this was a result of the foil burning rate increasing with pressure. The propellant ignited shortly after the foil burning surface passed by.

The burning rate of the propellant near the Al/PTFE foils depended on pressure, as represented in FIG. 12, as compared to a baseline propellant (without an accelerator) burning rate for reference. As pressure increased from 4.8 to 19.3 MPa, the enhanced burning rate near the Al/PTFE foils increased from six to ten times the burning rate of the bulk propellant. It is believed that the burning rate changes with pressure may have been due to changes in aluminum-fluorine reaction rates as pressure increased. The gasification of PTFE inside aluminum particles, as well as heating resulting in expansion, may cause pressures that break the aluminum apart during combustion (micro explosions). The aluminum particles produced from these types of materials are believed to be less than 10 microns in diameter when included in propellants, resulting in kinetically-limited combustion and stronger pressure sensitivity.

The investigations indicated that the Al/PTFE foil increased the propellant burning rate, as well as increased the propellant specific impulse. As an illustration, the copper, Ni/Al, and Pyrofuzer® wires and foils may be compared (to some extent) to catalysts in that they aid in combustion of the propellants but do not significantly participate reactively and remain as slag after the bulk propellant is consumed. On the other hand, aluminum (from the aluminum-rich MA Al/PTFE wire) contributes as a fuel in propellants to increase the specific impulse by increasing the combustion gas temperature.

It is believed that a propellant grain having an Al/PTFE accelerator may be locally more fuel-rich than a similar propellant grain with dispersed fuel. The PTFE may add some amount of fluorination to assist in the aluminum combustion. Additionally, the condensed phase products (slag) are predicted to be smaller than those of the other wires, which could result in lower two-phase flow losses. The mixture ratio of Al and PTFE could be varied to specifically tailor the enhanced burning rate. Further, milling parameters could be adjusted to change the foil burning rate. This gives the enhanced burning rates significant variability. Other similar mechanically-activated systems could also be considered.

Slag resulting from the copper wires (above) and Ni/Al foils (below) are represented in FIG. 13. No slag was collected from the propellant grains with Pyrofuzer® wire, but may be expected to be produced as combustion of the wire at 1 atm yielded spherical products of about 1 mm in diameter. Very occasionally, similarly sized spheres were seen embedded in the char covering the propellant window, but were not collected. From this point of view, the Pyrofuzer® wire may have benefits relative to the copper wires or the Ni/Al foils in fielded propellants as the condensed phase products are expected to be smaller, though slag size is

## 11

dependent in part on the amount of material used. No slag was observed for the Al/PTFE propellant grains.

In theory, the bulk propellant burning rate should only change in the area immediately surrounding the metallic fiber. To verify this assertion in the composite propellant environment, the lateral burning rate of the propellants after ignition was measured. In general, the bulk propellant burning rate did not significantly change after ignition. However, the bulk propellant burning rate of the grain having an embedded Pyrofuz® wire did change slightly (e.g., decreased) for unknown reasons.

While the invention has been described in terms of specific or particular embodiments and investigations, it should be apparent that alternatives could be adopted by one skilled in the art. For example, the propellant and its components could differ in appearance and construction from the embodiments described herein and shown in the drawings, the components of the reactive accelerator may differ from the nonlimiting examples described herein, and various materials could be used in the manufacturing of the propellant and its components. Accordingly, it should be understood that the invention is not necessarily limited to any embodiment described herein or illustrated in the drawings. It should also be understood that the phraseology and terminology employed above are for the purpose of describing the disclosed embodiments and investigations, and do not necessarily serve as limitations to the scope of the invention. Therefore, the scope of the invention is to be limited only by the following claims.

The invention claimed is:

1. A body having a bulk axis and comprising a solid energetic material and a reactive burning rate accelerator material at least partially embedded in and contacting the solid energetic material, the reactive burning rate accelerator material comprising at least one metallic component and at least one non-metallic component that are combined to form the reactive burning rate accelerator material and exothermally self-react to exothermically generate heat, wherein the reactive burning rate accelerator material is embedded in the solid energetic material as at least one foil or strand that extends within the solid energetic material in a bulk axial direction of the body so as to ignite and combust to increase the mass burning rate of the solid energetic material and so that combustion of the reactive burning rate accelerator material causes the solid energetic material to regress away from the at least one foil or strand and in the bulk axial direction of the body to create a continuous cone-shaped void within the solid energetic material that extends in the bulk axial direction of the body.

2. The body of claim 1, wherein the body is chosen from the group consisting of explosives, propellants, pyrotechnics, and fuels, the body further comprises an oxidizer and a binder that bonds the solid energetic material, the oxidizer, and the reactive burning rate accelerator material, and the reactive burning rate accelerator material combusts without an external oxidizer to produce a gas.

3. The body of claim 1, wherein the reactive burning rate accelerator material is a mechanically-activated material and the at least one foil or strand is at least partially formed of micron-sized particles comprising nano-thickness layers of the at least one metallic component and the at least one non-metallic component.

4. The body of claim 3, wherein the at least one metallic component comprises aluminum and the at least one non-metallic component comprises polytetrafluoroethylene.

5. The body of claim 1, wherein the at least one foil or strand of the reactive burning rate accelerator material

## 12

consists essentially of micron-sized particles comprising nano-thickness layers of the at least one metallic component and the at least one non-metallic component, wherein the at least one metallic component is aluminum and the at least one non-metallic component is polytetrafluoroethylene.

6. The body of claim 1, wherein the at least one metallic component comprises aluminum and the at least one non-metallic component comprises poly(carbon monofluoride).

7. The body of claim 1, wherein the at least one foil or strand of the reactive burning rate accelerator material consists essentially of micron-sized particles comprising nano-thickness layers of the at least one metallic component and the at least one non-metallic component, wherein the at least one metallic component is aluminum and the at least one non-metallic component is poly(carbon monofluoride).

8. The body of claim 1, wherein the reactive burning rate accelerator material comprises 50 to 90 wt. % of the at least one metallic component and 10 to 50 wt. % of the at least one non-metallic component.

9. The body of claim 1, wherein the reactive burning rate accelerator material comprises 70 to 90 wt. % of the at least one metallic component and 10 to 30 wt. % of the at least one non-metallic component.

10. A body having a bulk axis and comprising a solid energetic material and a reactive burning rate accelerator material at least partially embedded in and contacting the solid energetic material, the reactive burning rate accelerator material comprising a mechanically-activated material that

30 is at least partially formed of micron-sized particles comprising nano-thickness layers of at least one metallic component and at least one non-metallic component that exothermally self-react to exothermically generate heat, wherein the reactive burning rate accelerator material is embedded in the solid energetic material as at least one foil or strand that extends within the solid energetic material in a bulk axial direction of the body so as to ignite and combust to increase the mass burning rate of the solid energetic material and so that combustion of the reactive burning rate accelerator material causes the solid energetic material to regress away from the at least one foil or strand and in the bulk axial direction of the body to create a continuous cone-shaped void within the solid energetic material that extends in the bulk axial direction of the body.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795

15. The body of claim 10, wherein the reactive burning rate accelerator material comprises 70 to 90 wt. % of the at least one metallic component and 10 to 30 wt. % of the at least one non-metallic component.

16. A method of manufacturing the body of claim 10, the method comprising casting the reactive burning rate accelerator material within the solid energetic material. 5

17. A method of manufacturing the body of claim 10, the method comprising using a three-dimensional (3-D) printing process to insert the reactive burning rate accelerator material into the body. 10

\* \* \* \* \*